

# United States Patent [19]

Hiraki et al.

[11] Patent Number: 5,011,733

[45] Date of Patent: Apr. 30, 1991

[54] PROCESS FOR COATING METALLIC SUBSTRATE

[75] Inventors: Tadayoshi Hiraki; Osamu Iwase; Hiroshi Oosumimoto; Shinji Sugiura; Ichiro Tabushi; Masafumi Kume; Takashi Udagawa; Komaharu Matsui; Yasuhiro Fujii, all of Hiratsuka, Japan

[73] Assignee: Kansai Paint Co., Ltd., Hyogo, Japan

[21] Appl. No.: 296,343

[22] Filed: Jan. 9, 1989

## Related U.S. Application Data

[60] Continuation of Ser. No. 50,480, May 18, 1987, abandoned, which is a division of Ser. No. 907,212, Sep. 12, 1986, abandoned.

## Foreign Application Priority Data

Sep. 17, 1985 [JP] Japan 60-205065

[51] Int. Cl. 5 C25D 13/04; C25D 13/10; C25D 13/12; B32B 27/38

[52] U.S. Cl. 428/336; 204/181.1; 204/181.7; 427/410; 427/413; 427/417; 427/418; 427/419.1; 428/414; 428/416; 428/463; 428/494; 428/520; 428/521

[58] Field of Search 204/181.1, 181.7; 427/409, 410, 413, 417, 418, 419.1; 428/336, 416, 414, 463, 494, 520, 521

## [56] References Cited U.S. PATENT DOCUMENTS

|           |        |              |           |
|-----------|--------|--------------|-----------|
| 3,639,147 | 2/1972 | Benefiel     | 427/409   |
| 4,139,672 | 2/1979 | Ozawa et al. | 427/409   |
| 4,456,507 | 6/1984 | Kivel et al. | 204/181.1 |
| 4,463,038 | 7/1984 | Takeuchi     | 427/409   |
| 4,500,399 | 2/1985 | Hart         | 204/181.1 |
| 4,536,558 | 8/1985 | Kordomenos   | 204/181.7 |
| 4,755,418 | 7/1988 | DebRoy       | 209/181.1 |

Primary Examiner—T. Tung

Assistant Examiner—David G. Ryser

Attorney, Agent, or Firm—Wenderoth, Lind & Ponack

## [57] ABSTRACT

A process for coating a metallic substrate, characterized by applying on a metallic substrate a electrocoating paint, applying thereon a barrier coat comprising a film-forming thermoplastic resin other than a modified polyolefin resin and capable of forming a barrier coat film having a static glass transition temperature of 0° to -75° C., optionally applying on said barrier coat an intermediate coating paint and then applying thereon a top coating paint.

20 Claims, No Drawings

## PROCESS FOR COATING METALLIC SUBSTRATE

This application is a continuation, of now abandoned application Ser. No. 07/050,480, filed May 18, 1987, which is a Rule 60 divisional of Ser. No. 06/907,212, filed Sept. 12, 1986 now abandoned.

This invention relates to a process for coating a metallic substrate. More particularly, the present invention relates to a process for coating a metallic substrate such as, for example, a steel panel or the like constituting automotive bodies to form thereon a composite coating film excellent in chipping resistance, corrosion resistance, weather resistance and other physical properties.

Recently in the field of coating, there has come to be taken up more seriously the durability of the coating film on automotive outer bodies, particularly, the progress of corrosion of the metal materials of these outer bodies caused by the impact cracking of the coating film. For example in the cold climatic areas of Europe and America, in order to prevent the surface freezing of roads for automobiles, there are often laid on the roads in winter pebbles mixed with a large quantity of rock salt ground to relatively coarse particles. In automobiles running on such roads, the coating film on their outer portions is hit by the rock salt particles and pebbles flipped by the wheels and this impact often causes an impact cracking phenomenon, namely, so-called "chipping" in which the coating film locally peels off the body completely. Owing to this phenomenon, the metal surface of the outer body beneath the hit areas of the coating film is exposed to an atmosphere leading to rapid formation of rust and progress of corrosion. The cracking of coating film due to chipping ordinarily appears more in the bottom and underbody but it appears even in the hood or the roof. It is known that the resulting local corrosion progresses to a considerable degree in about 6 months to one year.

In order to prevent the chipping of coating film and the resulting progress of corrosion of the metal substrate beneath the coating film, there have heretofore been made various investigations on the chemical treatment, electrocoating primer, intermediate coating paint, and top-coating paint to be applied to the surface of metallic substrate of automotive outer body. For example, with respect to the chemical treatment, there was investigated the formation of an iron phosphate type film and a zinc phosphate type film each of different crystal form, but such a chemical treatment can not elevate the adhesivity of coating film to substrate metal to a level sufficiently resisting the impact of pebbles, etc. Also, with respect to the electrocoating paint and the top coating paint, various investigations were made on resins and/or pigments to be contained in these paints, but no electrocoating paint or top coating paint having an adhesivity sufficiently resisting the chipping has been developed yet.

There was also investigated the use of sericite or talc powder which is a foil-shaped inorganic pigment, in the composition of an intermediate coating paint. This method is intended to buffer and/or dissipating the impact applied to the coating film of automotive outer body, by a slipping action within the intermediate coating film due to the foil-shaped inorganic pigment, or to allow local peeling to occur only within the intermediate coating film or only at the interface between the electrocoating film and the intermediate coating film,

and consequently to prevent the electrocoating film from being damaged so that the electrocoating film can maintain a sufficient rust prevention function. However, this method has the following drawback. That is, since the impact applied to the outer surface of automotive body is varied and is fairly large in some cases, when there is applied such an impact as can not be softened or dissipated by the slippage within the intermediate coating film, the impact can not be completely absorbed by the intermediate coating film and spreads to all the coating film including the electrocoating film and, as a result, all the coating films at the portions which have received the impact peel off the metallic substrate, whereby rust develops quickly and corrosion progresses at these metallic substrate portions.

Hence, the present inventors made an extensive study in order to improve the above mentioned conventional drawbacks and to provide a process for coating a metallic substrate, particularly a steel panel to form thereon a multi-layered coating film excellent in chipping resistance, corrosion resistance, weather resistance and other physical properties and yet having a good film appearance as possessed by conventional coating systems for steel panels comprising an electrocoating paint, an intermediate coating paint which is optional, and a top coating paint. As a result, the present invention has been completed.

According to the present invention, there is provided a process for coating a metallic substrate, characterized by applying on a metallic substrate an electrocoating paint, applying thereon a barrier coat comprising a film-forming thermoplastic resin other than a modified polyolefin resin and capable of forming a barrier coat film having a static glass transition temperature of 0° to -75° C., optionally applying on said barrier coat an intermediate coating paint and then applying thereon a top coating paint.

An important characteristic of the present invention lies in that in a process for coating a metallic substrate, particularly a steel panel with an electrocoating paint, an optional intermediate coating paint and a top coating paint in this order, a barrier coat having a particular composition and a particular property is applied on the electrocoating film formed, prior to the application of the optional intermediate coating paint or the top coating paint. Due to the application of this barrier coat, the formation of a composite coating film very excellent in chipping resistance, corrosion resistance, weather resistance and other physical properties has become possible.

Thus, in the composite coating film formed according to the process of the present invention, since the barrier coat film contained therein at about its intermediate portion has flexibility and a unique visco-elasticity, even if the surface of the top coating film formed on or above the barrier coat film receives a strong impact of rock salt, pebbles, etc., the impact energy is mostly or completely absorbed within the barrier coat film and does not reach the electrocoating film beneath the barrier coat film and moreover even the top coating film and the optional intermediate coating film undergo little physical damage. That is, the barrier coat film has a buffer action for external impacts, whereby the chipping resistance of coating film system has been remarkably improved, development of rust and corrosion on steel panels caused by chipping has been prevented and the deterioration of the top coating film due to collision of rock salt, pebbles, etc. has been solved.

When the barrier coat film contains a corrosion-preventive pigment, the resulting composite coating film has significantly improved corrosion resistance as compared with when said pigment is contained in the electrocoating film.

The composite coating film formed according to the process of the present invention is very excellent also in such characteristics as film appearance, weather resistance, chemicals resistance and the like.

The coating process according to the present invention will be described in detail below.

#### Metallic substrate

This is a substrate material to be coated according to the present invention process. As the metallic substrate to which the present invention process is applicable, there can be used any materials having a metal surface to which cation electrocoating can be applied. Such materials include, for example, shaped articles made of iron, copper, aluminum, tin, zinc or an alloy thereof as well as products having a plated or deposited film of said metal or alloy. A steel panel is particularly preferred. Specifically, there are mentioned bodies and parts made of said materials, of passenger cars, trucks, safari cars, motor bicycles, etc. It is preferable that the surfaces of these metallic substrates be subjected to a chemical treatment with a phosphate, a chromate or the like prior to the application thereon of a cation type electrocoating paint.

#### Electrocoating Paint

This is an electrocoating paint to be applied on the surface of the above metallic substrate. As the electrocoating paint, both an anion type and a cation type can be used. The electrocoating paint of cation type is preferred.

[A] The cation type electrocoating paints include thermosetting electrocoating paints of cathodic deposition type wherein a base resin having basic amino groups is neutralized with an acid and dissolved (or dispersed) in water. These paints are coated on a metallic substrate using the substrate as a cathode.

A the resin having basic amino groups, there are suitably used resins generally having a base value of about 20 to about 200 obtained by, for example, (1) addition of an amine to epoxy groups (oxirane rings) of an epoxy group-containing resin such as a bisphenol type epoxy resin, an epoxy group-containing (or glycidyl group-containing) acryl resin, a glycidyl ether of alkylene glycol, an epoxidized polybutadiene, an epoxidized novolak phenol resin or the like; (2) polymerization using, as a monomer, an unsaturated compound having basic amino groups such as N,N-dimethylaminoethyl methacrylate, N,N-diethylaminoethyl acrylate, N-vinylpyrazole or the like; (3) reaction of a polyisocyanate compound with a glycol containing, as one component, a tertiary amino group-containing glycol (e.g. N-methyldiethanolamine); and (4) introduction of amino groups to a resin by an imidoamine formation reaction between an acid anhydride and a diamine.

The base value of a resin is mg of KOH corresponding to the equivalent of HCl required to neutralize 1 g of the resin.

As the amine used in the above reaction (1), there can be mentioned primary amines, secondary amines and tertiary amine salts of aliphatic type, alicyclic type and araliphatic type. Products obtained by adding to the epoxy group-containing resin mentioned in (1), a sec-

ondary sulfide salt or a tertiary phosphine salt in place of said amine can also be used in the present invention as a vehicle component of the cation type electrocoating paint.

5 As the neutralizing agent to neutralize the resin having basic amino groups to dissolve (or disperse) the resin in water, there can be used, for example, organic acids such as acetic acid, hydroxyacetic acid, propionic acid, butyric acid, lactic acid, glycine and the like as well as inorganic acids such as sulfuric acid, hydrochloric acid, phosphoric acid and the like. The appropriate amount of the neutralizing agent to the resin is about 0.1 to about 0.4 time the neutralization equivalent for the base value of the resin (generally about 20 to about 200).

10 As the crosslinking agent incorporated into the cation type electrocoating paint to make it thermosetting, there is generally used a blocked polyisocyanate compound. When the electrocoating paint is coated on a substrate and heated (ordinarily to 140° C. or a higher temperature), the crosslinking agent causes dissociation, whereby the isocyanate groups are regenerated and cause a crosslinking reaction with active hydrogen-containing functional groups (e.g. hydroxyl group) presnet in the resin having basic amino groups. Thus, the electrocoating paint coated becomes a cured film.

15 [B] Meanwhile, the anion type electrocoating paints include electrocoating paints of anodic deposition type wherein a base which is a carboxyl group-containing resin in most cases is neutralized with a basic compound 20 and dissolved (or dispersed) in water. These paints are 25 coated on a metallic substrate using the substrate as an anode.

30 As the carboxyl group-containing resin, there can be mentioned, for example, (1) maleinized oil resins obtained by addition of maleic anhydride to a drying oil (e.g. linseed oil, dehydrated castor oil, tung oil), (2) maleinized polybutadienes obtained by addition of maleic anhydride to a polybutadiene [e.g. a poly(1,2-butadiene), a poly(1,4-butadiene)], (3) resins obtained by 35 addition of maleic anhydride to an unsaturated fatty acid ester of an epoxy resin, (4) resins obtained by addition of a polybasic acid (e.g. trimellitic anhydride, a maleinized fatty acid, a maleinized oil) to a high molecular 40 polyalcohol having a molecular weight of about 1,000 or more (includes even partially esterified epoxy resins and styrene/allyl alcohol copolymers), (5) carboxyl group-containing polyester resins (include even such resins modified with a fatty acid), (6) carboxyl group-containing acrylic resins and (7) resins obtained by 45 addition of maleic anhydride to a (co)polymer formed from a reaction product between (a) a polymerizable unsaturated monomer having a glycidyl group or a hydroxyl group and (b) an unsaturated fatty acid. Of 50 these resins, those having a carboxyl group content of about 30 to 200 when expressed as an acid value are 55 suitable.

As the neutralizing agent used for neutralizing the carboxyl group of the carboxyl group-containing resin to make the resin soluble (or dispersible) in water, there 60 can be used, for example, alkanolamines such as monoethanolamine, diethanolamine, dimethylaminoethanol and the like; alkylamines such as diethylamine, triethylamine and the like; and inorganic alkalis such as potassium hydroxide, sodium hydroxide and the like. The appropriate use amount of the neutralizing agent is about 0.1 to 1.0 times, preferably 0.4 to 0.8 times the theoretical neutralization equivalent for the acid value of the carboxyl group-containing resin.

In order to provide the anion type electrocoating paint with curability, a low molecular melamine resin such as hexakis(methoxymethyl)melamine, butoxylated methylmelamine, ethoxylated methylmelamine or the like can be added to the paint as necessary as a cross-linking agent.

[C] Into the above mentioned cation or anion type electrocoating paint usable in the present invention are further incorporated, if necessary, pigments (e.g. a color pigment, an extender pigment, a corrosion-preventive pigment), hydrophilic organic solvents (e.g. isopropanol, n-butanol, ethoxyethanol, diethylene glycol monomethyl ether, diethylene glycol monoethyl ether, diethylene glycol monobutyl ether), water and ordinarily used additives. The resulting mixture is adjusted with a deionized water so as to have a solids content of about 5 to about 40% by weight and its pH is kept at 5.5 to 8.0 in the case of the cation type electrocoating paint and at 7 to 9 in the case of the anion type electrocoating paint.

The electrocoating paint thus prepared is subjected to electrocoating. It is usually conducted under conditions of 15° to 35° C. (bath temperature) and 100 to 400 V (load voltage) using a metallic substrate as a cathode in the case of the cation type electrocoating paint or as an anode in the case of the anion type electrocoating paint. The electrocoating film thickness is not particularly restricted and can vary largely depending upon the application of finished product, etc. However, the thickness is preferred to be generally 10 to 40  $\mu$ , particularly 15 to 35  $\mu$  in terms of cured film thickness of flat portions. The baking and curing temperature of the coating film is suitably 100° to 210° C. generally, and preferably 140° to 200° C. However, when there is used, in electrocoating, an anion type coating paint using, as its vehicle, an air-drying, unsaturated fatty acid-modified resin, the resulting coating film may be dried at room temperature.

In the preparation of the electrocoating paint, pigments have generally been used, in order not to reduce the smoothness of coating film, in an amount less than 40 parts by weight, ordinarily 35 parts by weight or less based on 100 parts by weight of resin solid. In the present invention, too, pigments can be used in the electrocoating paint in the above amount. However, it was found in the present invention that use of pigments in the electrocoating paint in an amount of 40 parts by weight or more based on 100 parts by weight of resin solid can give a final coated product whose metallic substrate (especially, its acute-angled portions) is further improved in corrosion resistance and chipping resistance.

Metallic substrate, for example, automotive bodies contain many acute-angled portions of steel panel such as side, bottom and back of facia, fender, door panel, panel hood, panel roof, panel trunk lid and body. Unlike other flat portions, these acute-angled portions have an acute-angled or projected shape. At such portions, paints do not adhere sufficiently and, once adhered, melt-flow during heat curing. Therefore, it has been inevitable that the film thickness gets thinner at the acute-angled portions as compared with that of flat portions and, especially at very acute-angled portions, the film thickness becomes extremely thin. As a result, the acute-angled portions have far inferior corrosion resistance than the flat portions and rust tends to easily appear firstly in the acute-angled portions. In contrast, when the present invention process is carried out using a cation or anion type electrocoating paint containing a

high concentration of pigments, the electrocoating paint adheres sufficiently even to the acute-angled portions and fine uneven portions present on the surface of the electrocoating film are filled by a barrier coat (to be described later), whereby the penetration of an intermediate coating paint or a top coating paint can be prevented and a coating system having improved surface smoothness, distinctness of image gross, corrosion resistance of acute-angled portions, etc. can be obtained.

The amount of pigment incorporated in the electrocoating paint in order to obtain such a coating system is more than in normal cases and specifically is 40 to 150 parts by weight, preferably 55 to 100 parts by weight, more preferably 60 to 85 parts by weight based on 100 parts by weight of resin solid. Needless to say, there can also be used in the present invention an amount less than 40 parts by weight ordinarily 35 parts by weight or less based on 100 parts by weight of resin solid which hitherto has been used generally. The pigments usable in the electrocoating paint are not particularly restricted in type and include color pigments, extender pigments, rust preventive pigments, etc. which are all known. As such pigments, there can be mentioned, for example, zinc oxide, antimony white, basic lead sulfate, basic lead carbonate, titanium dioxide, lithopone, lead silicate, zirconium oxide, carbon black, graphite, black iron oxide, aniline black, cuprous oxide, cadmium red, chrome vermillion, red iron oxide, pigment red, pigment violet, pigment orange, basic lead chromate, chrome yellow, ocher, cadmium yellow, strontium chromate, titanium yellow, litharge, pigment yellow, pigment green, zinc green, chrome green, chromium oxide, Phthalocyanine Green, ultramarine, prussian blue, Phthalocyanine Blue, pigment blue, cobalt violet, pigment violet, zinc powder, zinc oxide, red lead, lead cyanide, calcium plumbate, zinc yellow, silicon carbide, aluminum powder, asbestine, alumina, clay, diatomaceous earth, slaked lime, gypsum, talc, barium carbonate, precipitated calcium carbonate, calcium carbonate, precipitated barium sulfate, barite, bentonite, white carbon, glass beads, etc. These pigments can be used alone or in a combination of two or more.

#### Barrier coat

This is a composition to be applied on the surface of the electrocoating paint already applied. There is employed as the barrier coat a coating composition composed mainly of a film-forming thermoplastic resin other than a modified polyolefin resin and capable of forming a barrier coat film having a static glass transition temperature of 0° to -75° C., preferably -30° to -60° C., more preferably -40° to -55° C.

As the film-forming thermoplastic resin used as a vehicle in the barrier coat, there are preferably used those having excellent adhesivity not only to the previously mentioned electrocoating film but also to the intermediate or top coating film which will be explained later and capable of forming a barrier coat having a static glass transition temperature of the previously mentioned range. Specific examples of the film-forming thermoplastic resin are as follows.

#### (1) Styrene-butadiene copolymers

Styrene-butadiene copolymers having a styrene content of about 1 to 80% by weight, preferably 10 to 40% by weight. These copolymers can be produced by copolymerizing styrene and butadiene according to an ordinary method such as solution polymerization, suspen-

sion polymerization, emulsion polymerization, melt polymerization or the like.

Said styrene-butadiene copolymers can have a number-average molecular weight generally of about 10,000 to about 1,000,000, preferably 20,000 to 300,000.

#### (2) Polybutadienes

The polybutadienes usable in the barrier coat of the present invention can have a number-average molecular weight generally of 10,000 to 700,000, preferably 30,000 to 300,000.

These polybutadienes may comprise other comonomer such as acrylic acid, methacrylic acid or their alkyl ester, in such a small amount as the properties of said polybutadienes are not affected, for example, in an amount of 10% by weight or less.

#### (3) Acrylonitrile-butadiene copolymers

Acrylonitrile-butadiene copolymers having an acrylonitrile content of 1 to 50% by weight, preferably 10 to 40% by weight. These copolymers can be produced by copolymerizing acrylonitrile, butadiene and as necessary a small amount (e.g. 10% by weight or less) of other comonomer such as acrylic acid, methacrylic acid or their alkyl ester, according to an ordinary polymerization method such as solution polymerization, suspension polymerization, emulsion polymerization, melt polymerization or the like. In the case of emulsion polymerization, it is advantageous to use, as the other comonomer, a functional group-containing monomer such as acrylic acid, methacrylic acid or the like and to conduct emulsion polymerization in water in the presence of a polymerization catalyst, a molecular weight modifier, a surfactant, etc. The polymerization temperature employed at that time is preferred to be 100° C. or less generally.

The appropriate number-average molecular weight of said acrylonitrile-butadiene copolymers is ordinarily about 10,000 to about 1,000,000, preferably 30,000 to 300,000.

#### (4) Polybutenes

The polybutenes usable in the barrier coat are those produced by polymerizing isobutylene and as necessary a small amount of n-butylene at low temperatures.

These polybutenes have a number-average molecular weight ordinarily of about 1,000 to about 500,000, preferably 10,000 to 300,000.

The polybutenes can be made into an aqueous emulsion by heating such a polybutene to 50° to 70° C., adding thereto water and an emulsifier and then stirring them uniformly and thoroughly.

#### (5) Acrylic resins

Polymers obtained by copolymerizing an acrylic acid ester and/or a methacrylic acid ester and, as necessary, a small proportion, preferably 20% by weight or less, more preferably 15% by weight or less of at least one vinyl monomer selected from functional acrylic or methacrylic monomers and other polymerizable unsaturated monomers. These polymers can have a number-average molecular weight ordinarily of about 5,000 to about 1,000,000, preferably 50,000 to 300,000.

As the acrylic acid ester and the methacrylic acid ester, there can preferably be used C<sub>2</sub> to C<sub>20</sub> alkyl esters of acrylic acid or methacrylic acid whose homopolymers have a static glass transition temperature of 0° C. or lower, such as ethyl acrylate, isopropyl acrylate,

n-butyl acrylate, isobutyl acrylate, 3-pentyl acrylate, hexyl acrylate, 2-heptyl acrylate, octyl acrylate, 2-octyl acrylate, nonyl acrylate, lauryl acrylate, 2-ethylhexyl acrylate, 2-ethylbutyl acrylate, pentyl methacrylate, hexyl methacrylate, 2-ethylhexyl methacrylate, decyl methacrylate, lauryl methacrylate, stearyl methacrylate and the like. These esters can be used singly or as a combination of two or more. The amount of these esters whose homopolymers have a static glass transition temperature of -40° C. or lower, in the monomer mixture to be copolymerized is desired to be 30% by weight or more, preferably 60% by weight or more.

As the functional acrylic or methacrylic monomer which can be copolymerized as necessary with the acrylic acid ester and/or the methacrylic acid ester, there can be mentioned, for example, acrylic acid and methacrylic acid; C<sub>2</sub> to C<sub>10</sub> hydroxyalkyl esters of acrylic acid or methacrylic acid such as hydroxyethyl acrylate, hydroxypropyl acrylate, hydroxyethyl methacrylate, hydroxypropyl methacrylate and the like; amides of acrylic acid or methacrylic acid such as acrylamide, methacrylamide and the like; and glycidyl esters such as glycidyl acrylate, glycidyl methacrylate and the like.

As the other polymerizable unsaturated monomer which can be copolymerized as necessary with the acrylic acid ester and/or the methacrylic acid ester, there can be mentioned, for example, esters of acrylic acid or methacrylic acid whose homopolymers have a static glass transition temperature higher than 0° C., such as methyl acrylate, methyl methacrylate, ethyl methacrylate, propyl methacrylate, n-butyl methacrylate, isobutyl methacrylate and the like; and vinyl compounds such as styrene, acrylonitrile, vinyltoluene, vinyl chloride, vinyl acetate and the like.

The above mentioned monomers can be (co)polymerized according to an ordinary polymerization method such as solution polymerization, emulsion polymerization or the like to obtain an acrylic resin.

#### (6) Other resins

Natural rubber, polychloroprenes, methyl methacrylatebutadiene copolymers (butadiene content: 20 to 80% by weight, preferably 40 to 70% by weight), polyvinylidene chlorides etc. These resins can be used in a solution form but are often used in a latex form (natural rubber) or an aqueous emulsion form (resins other than natural rubber).

Of the various resins mentioned above, particularly preferable for use in the barrier coat of the present invention are resins selected from the above (1) to (5). Examples of such a preferable resin is a styrene-butadiene copolymer having a styrene content of 1 to 80% by weight and a number-average molecular weight of 10,000 to 1,000,000 and an acrylic resin having a number-average molecular weight of 50,000 to 300,000 and comprising 30% by weight or more of an alkyl ester of acrylic acid or methacrylic acid whose homopolymer has a static glass transition temperature of -40° C. or lower.

These vehicle resins are preferred to have by themselves a static glass transition temperature of 0° to -75° C.; however, this is not essential. What is essential is that a coating film formed by the barrier coat has the above static glass transition temperature. Accordingly, even if a vehicle resin used does not have the above static glass transition temperature by itself, the resin can provide a barrier coat capable of forming a coating film

having a static glass transition temperature of 0° to -75° C., by using the resin in combination with a modifier for static glass transition temperature. Such a modifier for static glass transition temperature include thickeners. As thickeners usable in the present invention process, there can be mentioned those having a good compatibility with the vehicle resin used, such as, for example, a rosin, a rosin ester, a hydrogenated rosin, a polyterpene resin, an ester gum, an epoxy-modified polybutadiene, an aliphatic epoxy resin of low molecular weight, an aliphatic bisphenol type epoxy resin of low molecular weight, a polyoxytetramethylene glycol, a silicone rubber, a polyvinyl ethyl ether and a polyvinyl methyl ether. These thickeners preferably have a static glass transition temperature generally of +20° C. to -70° C. These thickeners can be added even to a vehicle resin having a static glass transition temperature of 0° to -75° C. In this case, the coating film of the barrier coat obtained has a more desirable static glass transition temperature. The amount of the thickener used differs by the type thereof, the type of vehicle resin used, the required physical properties of coating film formed, etc. and can not be strictly specified. However, the amount is generally 1 to 50 parts by weight, preferably 5 to 30 parts by weight based on 100 parts by weight 25 of vehicle resin.

The coating film formed by the barrier coat according to the present invention has a static glass transition temperature of 0° to -75° C., preferably -30° to -60° C., more preferably -40° to -55° C. In addition, the coating film desirably has an elongation at break ordinarily of 200 to 1,000%, preferably 300 to 800%, more preferably 400 to 700% in an atmosphere of -20° C.

"Static glass transition temperature" and "elongation at break" used in the present specification and the appended claims refer to the values obtained from the following measurement methods.

#### Test sample

A barrier coat was applied on a tin plate so that the 40 final film thickness became 25  $\mu$ . Baking was conducted for 30 min. at 120° C., after which the coating film was isolated using an amalgam process. This film isolated was used as a test sample.

#### Measurement methods

For the above test sample, static glass transition temperature was measured using a differential scanning calorimeter (DSC-10 type manufactured by Daini Seikosha). For the same test sample, elongation at break was measured at -20° C. using a universal tensile tester with constant temperature bath (Autograph S-D type manufactured by Shimadzu Corp.). In this measurement, the sample length was 20 mm and the tensile speed was 20 mm/min.

The vehicle resin and if necessary, the thickeners are selected so as to give a barrier coat film having desired physical properties as mentioned previously.

The barrier coat composed mainly of a vehicle resin can be prepared in a form of organic solvent type paint or aqueous type paint. Such a barrier coat of organic solvent type can be prepared by dissolving or dispersing a vehicle resin and if necessary a modifier for static glass transition temperature in an organic solvent. As the organic solvent, there can be mentioned aromatic hydrocarbons such as benzene, toluene, xylene and the like; aliphatic hydrocarbons such as hexane, heptane, octane, decane and the like; chlorinated hydrocarbon

such as trichloroethylene, perchloroethylene, dichloroethylene, dichloroethane, dichlorobenzene and the like.

An aqueous barrier coat can be prepared by dispersing a vehicle resin as mentioned above in an aqueous medium by (1) neutralizing the resin with an acid or a base when the resin has a functional group which can be neutralized with an acid or a base or (2) using an appropriate dispersant such as an emulsifier, a surfactant or the like.

10 In order for the aqueous barrier coat to provide a coating film of good appearance, it is possible to add to the aqueous barrier coat an organic solvent having excellent compatibility with or excellent solubility for the vehicle resin contained in the aqueous barrier coat. As such an organic solvent, there can be mentioned, for example, aromatic hydrocarbons such as benzene, toluene, xylene and the like; aliphatic hydrocarbons such as hexane, heptane, octane, decane and the like; chlorinated hydrocarbons such as trichloroethylene, perchloroethylene, dichloroethylene, dichloroethane, dichlorobenzene and the like; ketone type solvents such as methyl ethyl ketone, diacetone alcohol and the like; alcohol type solvents such as ethanol, propanol, butanol and the like; and cellosolve type solvents such as methyl cellosolve, butyl cellosolve, cellosolve acetate and the like.

When a top coating paint is directly applied on the barrier coat film (an intermediate coating paint is not applied), it is preferable that the barrier coat contains, 30 another organic solvent having a boiling point of 150° C. or higher and compatible with a top coating paint powder (hereinunder this organic solvent is referred at times to as "compatible solvent"), such as diisopropylbenzene, tetralin, decalin, o-dichlorobenzene, trichlorobenzene, benzyl alcohol, diisobutyl ketone, isophorone, cellosolve acetate, carbitol acetate, dimethyl phthalate or the like. Use of such a compatible solvent is preferable for the following reason. That is, when a barrier coat obtained by dissolving or dispersing a vehicle resin in a mixed solvent consisting of an organic solvent or water and a compatible solvent is applied and subsequently a top coating paint powder is applied on the still wet (not baked) barrier coat film and baked, the compatible solvent remaining in the barrier coat film evaporates and reaches the top coating powder film, whereby the resin powder has an improved melt-flow characteristics and the smoothness of finished coating surface is remarkably improved. The amount of compatible solvent in mixed solvent has no particular restriction but is preferably 5 to 50% by weight. The content of mixed solvent in barrier coat is appropriately 15 to 95% by weight. Thus, when a top coating paint powder is directly applied on a barrier coat film and an intermediate coating paint is not applied, by applying a top coating paint powder on a barrier coat film which is still wet and contains a compatible solvent, there can be effectively produced a finished coating surface having improved smoothness.

55 Into the barrier coat can be incorporated various additives if necessary. For example, there can be incorporated pigments mentioned with respect to the cation type electrocoating paint, such as color pigments, extender pigments corrosion-preventive pigments and the like (rust preventive pigments are excluded). The amount of pigments incorporated can be generally 150 parts by weight or less, preferably 100 parts by weight 60 or less based on 100 parts by weight of vehicle resin.

Particularly, a corrosion-preventive pigment is blended into the barrier coat, which is effective for markedly improving the corrosion resistance of the coating film formed by the present invention.

The corrosion-preventive pigment which can be incorporated into the barrier coat refers to the pigment which has the function of inhibiting or preventing corrosion of metals, and is clearly distinguished from coloring pigments for simply imparting color and extender pigments for adjusting the physical properties of the coating film. As examples of such corrosion-preventive pigment, lead-type pigments, chromate-type pigments, metallic powder pigments. The type of usable corrosion-preventive pigment is not particularly limited, but suitable ones are those having such a composition that, upon contact with water, of which corrosion-preventive component is eluted. Particularly preferred corrosion-preventive pigments are those of which extracts with water show electroconductivity of at least 100  $\mu$  U/cm, particularly at least 300  $\mu$  U/cm.

The electroconductivity of aqueous extract of a corrosion-preventive pigment is measured as follows: 80 parts by weight of deionized water having electroconductivity of not higher than 1  $\mu$  U/cm and 20 parts by weight of the corrosion-preventive pigment are mixed and allowed to stand for 5 days at 30° C. (In the meantime, the mixture is mixed for 10 minutes per day). Then the supernatant liquid (aqueous extract) is separated and its electroconductivity is measured.

Examples of corrosion-preventive pigments having electroconductivity within the above-specified range include zinc chromate (1570  $\mu$  U/cm), strontium chromate (973  $\mu$  U/cm), barium chromate (736  $\mu$  U/cm), calcium chromate (8000  $\mu$  U/cm), basic lead chromate (111  $\mu$  U/cm), base lead sulfate (118  $\mu$  U/cm), calcium phosphate (332  $\mu$  U/cm), zinc molybdate (333  $\mu$  U/cm), calcium molybdate (256  $\mu$  U/cm), aluminum phosphomolybdate (182  $\mu$  U/cm), barium metaborate (1540  $\mu$  U/cm), ammonium metavanadate (7450  $\mu$  U/cm) and the like. (The numerical values in the parentheses indicate the respective electroconductivity.) More than one of those can be used concurrently. Of those, particularly preferred are zinc chromate, strontium chromate, barium chromate and calcium chromate. The suitable amount of use of such corrosion-preventive pigment ranges 1-150 parts by weight, preferably 2-50 parts by weight, per 100 parts by weight of the vehicle resin.

Such advance blending of corrosion-preventive pigment with the barrier coat can markedly improve the corrosion resistance of the coating system, as compared with the cases wherein the pigment is blended with the electrocoating paint.

In order for the corrosion-preventive pigment contained in the barrier coat to fully exhibit its corrosion resistance, it is preferred that the water absorption of the electrocoating film is adjusted at 0.3 to 20% by weight, particularly 0.5 to 5% by weight.

The "water absorption" of the electrocoating film is a value calculated as follows. An electrocoating paint is applied onto a substrate to a cured film thickness of 20  $\mu$  (applied area: 5×5 cm) and baked under the conditions suitable for the components therein; the resulting coating film is isolated and immersed in warm water of 50° C. for 48 hours; its weight immediately after withdrawal from the water and that after drying it at 105° C. for 1 hour are measured; and the two weights obtained are inserted into the following equation.

$$5 \quad \text{Water absorption of coating film} = \frac{\text{film weight immediately after withdrawal from warm water} - \text{film weight after drying}}{\text{film weight after drying}} \times 100$$

- 10 Adjustment of the water absorption of the electrocoating film as above presumably facilitates the penetration of the water-extracted component of the corrosion-resistant pigment from the barrier coat containing said pigment into the electrocoating film, to fully exhibit its cathode- (or anode-) inhibiting effect on the surface of steel member and to protect the steel member. The 15 adjustment of water absorption can be easily effected by controlling the crosslinking density of the coating film, introduction of hydrophilic groups into the vehicle resin and the amount of blending extender pigment, or the like.
- 20 The adjustment of water absorption as mentioned above makes it unnecessary to add a corrosion-preventive pigment to the electrocoating paint. As a result, the electrocoating paint can have improved storage stability, film smoothness, etc.
- 25 Into the barrier coat can further be incorporated, for purposes of, for example, (1) improvement of physical properties of coating film, (2) improvement of dispersibility of pigments and (3) filling, etc., proper amounts of known additives for coatings such as, for example, a 30 rosin, a rosin ester, a hydrogenated rosin, a polyterpene resin, an ester gum, an epoxy-modified polybutadiene, an aliphatic epoxy resin of low molecular weight, an aliphatic bisphenol type epoxy resin of low molecular weight, a polyoxytetramethylene glycol, a silicone rubber, a polyvinyl ethyl ether, a polyvinyl methyl ether, a plasticizer (e.g. diethyl phthalate, tricresyl phosphate), an antisagging agent (e.g. aluminum stearate, silica gel), a pigment dispersing agent, a film surface improver and the like.
- 35 40 When an intermediate coating paint is omitted and a top coating paint is directly applied on the barrier coat film, it is preferable that the barrier coat further contains deterioration inhibitors for resins such as an ultraviolet absorber, a photostabilizer, an anti-oxidant and the like. The purpose of using such inhibitors is to absorb an ultraviolet rays passing through a top coating film having a small hiding power and to prevent the oxidation of radicals generated in resin chains and thereby to protect the barrier coat film and even the electrocoating film surface from being deteriorated with time by the ultraviolet ray.
- 45 The ultraviolet absorber usable in the barrier coat can be any as long as it can absorb the energy of ultraviolet ray, is compatible with or uniformly dispersible in the vehicle resin used in the barrier coat and does not easily decompose and lose its function at a temperature at which the barrier coat film or a whole coating system is baked. The usable ultraviolet absorber includes, for example, benzophenones such as benzophenone, 2,4-dihydroxybenzophenone, 2,2',4,4'-tetrahydroxybenzophenone, 2-hydroxy-4-methoxybenzophenone, 2,2'-dihydroxy-4,4'-dimethoxybenzophenone, 2,2'-dihydroxy-4-methoxybenzophenone, 2-hydroxy-4-octoxybenzophenone, 2-hydroxy-4-dodecyloxybenzophenone, 2-hydroxy-4-methoxy-5-sulfobenzophenone, 5-chloro-2-hydroxybenzophenone, 2,2'-dihydroxy-4,4'-dimethoxy-5-sulfobenzophenone, 2-hydroxy-4-methoxy-2'-carboxybenzophenone, 2-hydroxy-4-(2-
- 50 55 60 65

hydroxy-3-methylacryloxy)propoxybenzophenone and the like; benzotriazoles such as 2-(2'-hydroxy-5'-methylphenyl)benzotriazole, 2-(2-hydroxy-3,5-di(1,1-dimethylbenzylphenyl)-2H-benzotriazole, 2-(2'-hydroxy-3',5'-diteriary-butylphenyl)-benzotriazole, 2-(2'-hydroxy-3'-tertiary-butyl-5'-methylphenyl)benzotriazole, 2-(3,5-diteriary-amyl-2-hydroxyphenyl)benzotriazole, 2-(2'-hydroxy-3',5'-diteriary-butylphenyl)-5-chlorobenzotriazole, 2-(2'-hydroxy-3',5'-diteriaryisoamylphenyl)benzotriazole, 2-(hydroxy-5-tertiary-butylphenyl)benzotriazole and the like; salicylic acid esters such as phenyl salicylate, 4-tertiary-butylphenyl salicylate, p-octylphenyl salicylate and the like; diphenyl acrylates such as ethyl-2-cyano-3,3'-diphenyl acrylate, 2-ethylhexyl-2-cyano-3,3'-diphenyl acrylate and the like; hydroxy-5-methoxyacetophenone; 2-hydroxynaphthophenone; 2-ethoxyethyl-p-methoxycinnamate; nickel bisoctylphenylsulfide; [2,2'-thiobis(4-t-octylphenolate)-n-butylamine-nickel; oxalic acid anilide; etc. There are commercially available ultraviolet absorbers. As commercial products of benzotriazole type, there are mentioned, for example, Tinuvin 900 and Tinuvin 328, both of CIBA-Geigy Co. As products of benzophenone type, there is mentioned, for example, Unimul 400 (a product of BASF). As products of oxalic acid anilide type, there is mentioned, for example, Sanduvor 3206 of SANDOZ Ltd.

The amount of ultraviolet absorber used is preferably 0.1 to 10 parts by weight, more preferably 0.5 to 5 parts by weight based on 100 parts by weight of vehicle resin.

As the photostabilizer, there are mentioned, for example, tetrakis(2,2,6,6-tetramethyl-4-piperidyl) 1,2,3,4-butanetetracarboxylate, 8-acetyl-3-dodecyl-7,7,9,9-tetramethyl-1,3,8-triazaspiro(4,5)decane-2,4-dione, bis(1,2,2,6,6-entamethyl-4-piperidinyl) sebacate, bis(2,2,6,6-tetramethyl-4-piperidyl) sebacate, bis(1,2,2,6,6-pentamethyl-4-piperidyl) sebacate, dimethyl-2-(4-hydroxy-2,2,6,6-tetramethyl-1-piperidyl) ethanol condensate, poly-6-(1,1,3,3-tetramethylbutyl)imino-1,3,5-triazine-2,4-diyl-4-(2,2,6,6-tetramethylpiperidyl)-hexamethylene-4,4-(2,2,6,6-tetramethylpiperidyl-jimino), 1,2,3-(3,5-di-t-butyl-4-hydroxyphenyl)propionyloxyethyl]-3,4-(3,5-di-t-butyl-4-hydroxyphenyl)-propionyloxy-2,2,6,6-tetramethylpiperidine, etc. As the anti-oxidant, there are mentioned, for example, 4,4'-thiobis(3-methyl-6-t-butylphenyl), 2,2'-methylenebis(4-methyl-6-t-butylphenol), 4,4'-methylenebis(2,6-di-t-butylphenol), 1,3,5-trimethyl-2,4,6-tris(3,5-di-t-butyl-4-hydroxybenzyl)benzene, tris(2-methyl-4-hydroxy-5-t-butylphenyl)butane, pentaerythritol tetrakis(3-lauryl-thiopropionate), dilaurylthio dipropionate, distearylthio dipropionate, dimyristylthio dipropionate, triethylene glycol bis-3-(3-t-butyl-5-methyl-4-hydroxyphenyl)propionate, 1,6-hexanediol bis-3-(3,5-di-t-butyl-4-hydroxyphenyl)propionate, 2,4-bis(n-octylthio)-6-(4-hydroxy-3,5-di-t-butylanilino)-1,3,5-triazine, pentaerythritol tetrakis-3-(3,5-di-t-butyl-4-hydroxyphenyl)-propionate, 2,2-thiodiethylene-bis-3-(3,5-di-t-butyl-4-hydroxyphenyl)-propionate], octadecyl-3-(3,5-di-t-butyl-4-hydroxyphenyl)-propionate, 2,2-thiobis(4-methyl-6-t-butylphenyl), N,N'-hexamethylenebis(3,5-di-t-butyl-4-hydroxy-hydroxycinnanamide), etc. The photostabilizer and/or the anti-oxidant is used preferably in combination with the ultraviolet absorber. The appropriate amount of photostabilizer used is 0.1 to 10 parts by weight, preferably 0.5 to 3 parts by weight, based on 100 parts by weight of resin. The appropriate amount of

anti-oxidant used is 0.1 to 5 parts by weight, preferably 0.2 to 3 parts by weight on the same basis.

As one important requirement, the barrier coat film must have excellent adhesivity to the electrocoating film and the intermediate or top coating film which will be explained later. Desirably, the adhesivity to each of said films is at least 25 kg/cm<sup>2</sup>. The adhesivity is, by definition, a measurement by a tensile tester of an energy (kg/cm<sup>2</sup>) required to peel an attachment bonded to the barrier coat film on the electrocoating film or to the intermediate or top coating film on the barrier coat film. The adhesivity is measured by applying and curing each paint under predetermined conditions, bonding an attachment having a circular contact area of 5 mm in diameter to the resulting barrier coat film, intermediate coating film or top coating film using a two-pack epoxy resin adhesive, peeling the attachment from the film in a vertical direction at 20° C. at a tensile speed of 50 mm/min using a Schopper tensile tester manufactured by Ueshima Seisakusho and measuring a force (kg/cm<sup>2</sup>) required for the peeling.

The adjustment of the above mentioned adhesivity of the barrier coat film can be effected mainly by the selection of the type, amount, etc. of the vehicle resin contained in the barrier coat. It can also be effected by, for example, the addition of the above mentioned modifier or pigments.

In the present invention, the barrier coat can be applied either after the electrocoating film has been cured with heating or before said film is cured.

The application of the barrier coat on the electrocoating film already formed according to the method mentioned above can be conducted according to any known method such as spray coating, brush coating, dip coating, melt coating, electrostatic coating or the like. The film thickness of the barrier coat is preferred to be ordinarily 1 to 20 μ, particularly 2 to 10 μ in terms of thickness of dried film.

As mentioned previously, in the present invention process, on the surface of the barrier coat film formed is then coated an intermediate coating paint or a top coating paint. Prior to this coating, the barrier coat film can be baked. The prior baking is generally preferable but is not essential. Depending upon the type of paint to be applied on the barrier coat film, for example, when a top coating paint powder is directly applied on the barrier coat film, baking of the barrier coat film is not required and wet-on-wet application of an intermediate coating paint or a top coating paint is possible. There are cases that this wet-on-wet application is preferable.

The appropriate baking temperature is generally 80° C. to 200° C., particularly 80° to 160° C..

#### Intermediate coating paint

Onto the surface of the barrier coat film can be applied an intermediate coating paint, prior to the application of a top coating paint. The main purpose of conducting this intermediate coating is to allow a final coating film to have a high quality excellent in durability, surface smoothness and sharpness, adhesion, etc. Therefore, when the final coating film is not required to have such a high quality, the intermediate coating can be omitted.

As the intermediate coating paint optionally usable in the present invention process, there can be used any known intermediate coating paint which has been used in conventional coating systems consisting of a primer, an intermediate coating paint and a top coating paint

and is excellent in adhesion, distinctness of image gloss (surface smoothness), surface sharpness, overbaking resistance, weather resistance, etc. Specifically, there can be mentioned thermosetting intermediate coating paints using, as a vehicle main component, a combination of (1) a short or ultra-short oil alkyd resin having an oil length of 30% or less and/or an oil-free polyester resin and (2) an amino resin. The alkyd resin and the polyester resin desirably have a hydroxyl value ordinarily of 60 to 140, particularly 80 to 120 and an acid value of 5 to 100.

As the particularly preferable alkyd resins and polyester resins, there can be mentioned resins obtained from esterification between a polyhydric alcohol (e.g. ethylene glycol, propylene glycol, butylene glycol, hexanediol, neopentyl glycol, glycerine, trimethylolethane, trimethylolpropane, pentaerythritol) and a polybasic acid (e.g. phthalic acid, maleic acid, terephthalic acid, adipic acid, tetrahydroxyphthalic acid, fumaric acid, itaconic acid, pyromellitic acid, their anhydrides).

As the oil usable for modification of the alkyd resin, there can be mentioned, for example, drying oils or semi-drying oils such as linseed oil, soybean oil, safflower oil, tung oil, tall oil, dehydrated castor oil and the like, as well as unsaturated fatty acids obtained from said oils.

As the amino resin used in combination with the oil-modified alkyd resin or the oil-free polyester resin, generally there are suitably used melamine resins etherified with an alkyl group of 1 to 5 carbon atoms, urea resins, benzoguanamine resins, etc. With respect to the amount ratio of the amino resin to other resins, it is desirable that the oil-modified alkyd resin and/or the oil-free polyester resin is 65 to 85%, preferably 70 to 80% in terms of solid weight and the amino resin is 35 to 15%, preferably 30 to 20%. At least part of the amino resin can be replaced by a polyisocyanate compound or a blocked polyisocyanate. As the blocked or non-blocked polyisocyanate compound, there can be mentioned, for example, tolylene diisocyanate, diphenyl methane diisocyanate, xylylene diisocyanate, hexamethylene diisocyanate, isophorone diisocyanate, a reaction product between 1 mole of trimethylolpropane and 3 moles of tolylene diisocyanate or hexamethylene diisocyanate.

The intermediate coating paint using the above resins as vehicle components preferably has a form of organic solvent type or aqueous type (aqueous solution or aqueous dispersion). The organic solvent type is most preferable. The intermediate coating paint may also have a form of non-aqueous dispersion type, high solid type, powder type or the like. It is preferable that the intermediate coating paint give a coating film having a pencil hardness generally of 3B to 6H, preferably B to 2H at 20° C. The intermediate coating paint can further contain, if necessary, extender pigments, color pigments and other additives ordinarily used for coatings, in amounts ordinarily used.

The application of the intermediate coating paint on the barrier coat film can be conducted, as in the application of the barrier coat, using a method such as spray coating, brush coating, dip coating, melt coating, electrostatic coating or the like. It is preferable that the intermediate coating film have a thickness generally of 10 to 100  $\mu$ , preferably 15 to 50  $\mu$ . The curing of the intermediate coating film can be conducted at any temperature suitable for the curing characteristic of the film as long as the temperature causes no substantial thermal

deterioration of the film. However, when thermal curing is applied, the curing temperature is preferably 80° to 170° C., more preferably 120° to 150° C.

#### Top coating paint

This is a paint to be applied on the surface of the barrier coat film or of the intermediate coating film in order to give the coated bodies pleasant appearance. As this top coating paint, there can be used top coating paints used in conventional coating systems consisting of a primer, an intermediate coating paint and a top coating paint. As such top coating paint, there can generally be used conventionally known paints capable of forming a coating film excellent in surface appearance (e.g. sharpness, smoothness, gloss), weather resistance (e.g. gloss retention, color retention, chalking resistance), chemical resistance, moisture resistance, water-resistance, curability, etc. As the top coating paint usable in the present invention process, there can be mentioned, for example, crosslinking curable paints preferably of organic solvent type or aqueous type, using as the main vehicle component, a resin such as an amino-acryl resin type, an acid-glycidyl-acryl resin type, an isocyanate-acryl resin type, an unsaturated acryl resin type, an amino-alkyd resin type, an amino-polyester resin type, an amino-fluorinated resin type, an amino-silicone polyester resin type, an unsaturated polyester resin type, an isocyanate-polyester resin type, isocyanate-fluorinated resin type or the like.

Preferable examples of the top coating paint include an amino acryl resin type paint, namely, a thermosetting paint using an amino resin as a crosslinking agent. This paint uses, as main components, (a) an acryl resin obtained by polymerizing an appropriate combination of a hard monomer (e.g. methyl methacrylate, ethyl methacrylate, n-butyl methacrylate, isobutyl methacrylate), a soft monomer (e.g. n-hexyl methacrylate, lauryl methacrylate, methyl acrylate, ethyl acrylate, n-butyl acrylate, 2-ethylhexyl acrylate), a functional group-containing monomer (e.g. acrylic acid, methacrylic acid, hydroxethyl methacrylate, hydroxyethyl acrylate, acrylamide, glycidyl acrylate) and other monomer (e.g. styrene, acrylonitrile) and (b) an amino resin selected from resins such as a melamine resin etherified with an alkyl group of 1 to 5 carbon atoms and an urea resin etherified with an alkyl group of 1 to 5 carbon atoms. Said acryl resin (a) preferably has a number average molecular weight of 5,000 to 50,000, a hydroxyl value of 5 to 40 and an acid value of 2 to 100. Another preferable example of the top coating paint is an amino alkyd resin type paint, wherein a butylated melamine resin is preferable as the amino resin component and an alkyd resin modified with a semi-drying oil or an ultra-short oil alkyd resin is preferable as the alkyd resin component.

When the top coating paint is particularly a paint capable of forming an ultra-hard film, the composite coating film formed in accordance with the present invention process has a remarkably improved scuff resistance and is hard and flexible. This composite coating film, since its uppermost layer is an ultra-hard film and accordingly is hard, can almost completely prevent the formation of scuffs caused by a car washing brush, a polishing compound, dust, etc. and possesses improved weather resistance. Further, the composite coating film, since it also contains barrier coat film having physical properties as mentioned previously beneath or below the uppermost layer, even if it receives a strong impact force by collision of rock salt, pebbles, etc. at the

outermost ultra-hard film, can absorb completely or almost completely the impact energy within the barrier coat film; thereby, the impact energy does not reach the electrocoating film beneath the barrier coating film and yet the top coating film (and the intermediate coating film) receive little physical damage. That is, the barrier coat film functions as a buffer zone for impacts applied from outside, whereby the multi-layered coating film has remarkably improved chipping resistance, the metallic substrate such as a steel panel can be protected from development of rust and corrosion caused by chipping, and the top coating film can be free from damage by collision of rock salt, pebbles, etc. Thus, the multi-layered coating film is hard and flexible and accordingly exhibits excellent performances as mentioned above.

"Ultra-hard film" said herein is a coating film having a hardness (as cured) of 4H to 9H at 20° C. when measured in accordance with a pencil hardness testing method.

The pencil hardness testing method used in the present invention is such that a glass plate is coated with a paint to be tested according to the present invention process, the resulting composite coating film is cured, the resulting test plate is kept at 20° C., a pencil ("Uni" for drawing use, manufactured by Mitsubishi Pencil Ltd.) whose lead tip has been ground flatly so as to have a sharp edge is strongly pressed onto the coated surface of the test plate at an angle of 45° at such a pressure as the pencil lead is not broke, in this condition the pencil is moved by about 1 cm at a speed of 3 sec/cm, and in this way there is measured the hardness of the hardest pencil causing no scratch.

As the top coating paint capable of forming an ultra-hard film, there can be mentioned, for example, cross-linking-curable paints using, as a vehicle component, a resin such as an amino-acryl resin type, an amino-alkyd resin type, an amino-polyester resin type, an amino-fluorine resin type, an amino-silicone-polyester resin type, an unsaturated polyester resin type, an isocyanate-acryl resin-type, an isocyanate-polyester resin type, an isocyanate-fluorine resin type, an unsaturated acryl resin type or the like. Preferable of these are top coating paints of amino-alkyd resin type, amino-acryl resin type, and amino-silicon-polyester resin type.

As the method for forming an ultra-hard film, there can be mentioned, for example, (1) when the vehicle component is a polyester resin- or an alkyd resin-based, a method wherein the polybasic acid component of said resin is a hard, aromatic type polybasic acid such as phthalic acid, isophthalic acid, terephthalic acid, trimellitic acid, their anhydrides or the like, (2) when the vehicle component is an acryl resin-based, a method wherein said resin is a hard, acrylic type resin using a monomer giving a high glass transition temperature and (3) a method wherein the vehicle component is a resin having a relatively large molecular weight and containing within the molecule a large proportion of crosslinkable functional groups and the amount and type of catalyst (internal or external catalyst) and/or the amount and type of crosslinking agent (or curing agent) are controlled.

The form of the top coating paint used in the present invention process has no particular restriction and can be of organic solution type, non-aqueous dispersion type, aqueous solution type, aqueous dispersion type, powder type, high solid type, etc.

The top coating paint used in the present invention process is classified into (1) an enamel paint obtained by adding, to a paint using the above mentioned main vehicle component, metallic pigments and/or color pigments and (2) a clear paint completely or substantially free from these pigments. Using such a paint, a top coating film can be formed thermally according to, for example, the following methods.

- (1) A metallic paint containing metallic pigments and, as necessary, color pigments or a solid color paint containing color pigments is applied and heat-cured. (Metallic or solid color finishing by one coating and one baking)
- (2) A metallic paint or a solid color paint is applied and heat-cured. Then, a clear paint is applied and again heat-cured. (Metallic or solid color finishing by two coatings and two bakings)
- (3) A metallic paint or a solid color paint is applied and then a clear paint is applied. Subsequently, the resulting two films are cured simultaneously. (Metallic or solid color finishing by two coatings and one baking)

The top coating paints mentioned above are applied preferably by spray coating, electrostatic coating, etc. The resulting coating film is dried and/or cured by room temperature drying, heat drying, heat curing, crosslinking curing by irradiation of active energy rays (e.g. electron rays, ultraviolet rays), etc., depending upon the form, type, etc. of paint applied.

The top coating film formed as above preferably has a thickness (as dried) of 25 to 40  $\mu$  when the method (1) is used and 10 to 30  $\mu$  (metallic and solid color paints) and 25 to 50  $\mu$  (clear paint) when the method (2) or (3) is used. The heating condition of the top coating film can vary depending upon the type of vehicle component used. However, preferably it is generally 80° to 170° C., particularly 120° to 150° C. and 10 to 40 min.

When a top coating paint of powder type is mainly used as the top coating paint, there can be used, for example, the following coating and baking methods.

- (a) An enamel solid color paint of powder form obtained by adding color pigments to the vehicle component of the above mentioned powder paint is applied on the barrier coat film and baked. (Solid color finishing by one coating and one baking)
- (b) A solid color or metallic paint of liquid form is applied on the barrier coat film. Then, after or without baking, the above mentioned clear paint of powder form substantially or completely free from color pigments is applied and baking is conducted. (A solid color or metallic finishing by two coatings and one baking or by two coatings or two bakings)

In the method (a), after the barrier coat film has been baked, preferably a barrier coat containing a compatible solvent is applied. Thereon, without baking, is applied a solid color enamel paint of powder form so that this application can give a film having a thickness (after baking) of about 30 to 150  $\mu$ . The resulting film is baked at 120° to 210° C., particularly 130° to 180° C. By allowing the barrier coat film to contain a compatible solvent, the development of fine unevenness (as seen on orange skins) on the surface of the top coating film can be prevented and the top coating film can have an appearance of excellent smoothness.

In the method (b), a barrier coat is applied and, after or without baking, a solid color or metallic paint of liquid form is applied thereon so that the latter application can give a film having a thickness (after baking) of

10 to 30  $\mu$ . Then, after baking at, for example, 80° to 170° C. or without baking, the above mentioned clear paint of powder form is applied so as to give a film having a thickness (after baking) of 30 to 150 and baking is conducted at 80 to 170° C., particularly 120° to 160° C.

The top coating film formed can have a pencil hardness generally of 3B or greater, particularly 1H to 9H at 20° C., depending upon factors such as the type of vehicle component contained in the film.

The coating film formed as above according to the present invention process is excellent in surface appearance (e.g. smoothness, gloss, sharpness), water resistance, weather resistance, etc. and is remarkably improved particularly in chipping resistance and other physical (mechanical) properties. Accordingly, it is suitable for use particularly in automotive bodies.

The present invention will be more specifically described hereinbelow, with reference to Examples and Comparative Examples.

### I Samples

#### (1) Metallic substrates

(A) A steel panel treated with a surface treating agent of zinc phosphate type (dimensions: 30 mm × 90 mm × 0.8 mm).

(B) A steel panel having an acute-angled portion obtained by bending the steel panel (A) by 90°.

#### (2) Cation type electrocoating paints

(A) A paint using, as vehicle components, a polyamide-modified bisphenol type epoxy resin (acetic acid used as a neutralizing agent) and a blocked polyisocyanate compound. pH: 6.5 Solid content: 20% by weight.

(B) A paint comprising 100 parts by weight of the vehicle components of the paint (A) and 61.5 parts by weight of pigments consisting of 30 parts by weight of titanium dioxide, 1.5 parts by weight of carbon black and 30 parts by weight of clay. pH: 6.5 Solid content: 20% by weight. The coating film obtained by this paint alone was not satisfactory in smoothness.

(C) A paint comprising 100 parts by weight of the vehicle components of the paint (A) and 79 parts by weight of the pigment of the paint (B). pH: 6.5 Solid content: 20% by weight. The coating film obtained by this paint alone was inferior in smoothness.

#### (3) Barrier coats

(A) An aqueous dispersion obtained by emulsion-polymerizing a monomer mixture consisting of 30% by weight of styrene and 70% by weight of butadiene according to an ordinary method. Static glass transition temperature: -48° C., elongation at break at -20° C.: 450%.

(B) An aqueous dispersion obtained by adding 10 parts by weight of barium chromate as a corrosion-preventive pigment to 100 parts by weight of an emulsion polymer of a composition consisting of 60% by weight of nonyl acrylate, 20% by weight of 2-ethylhexyl acrylate, 15% by weight of methyl acrylate and 5% by weight of hydroxyethyl acrylate. Static glass transition temperature: -48° C., elongation at break at -20° C.: 370%.

(C) An aqueous dispersion consisting only of the emulsion polymer of the above (B).

(D) An aqueous dispersion of an emulsion polymer of a composition consisting of 10% by weight of ethyl acrylate, 25% by weight of 2-octyl acrylate, 5% by

weight of hydroxyethyl methacrylate and 60% by weight of lauryl methacrylate. Static glass transition temperature: -52° C., elongation at break at -20° C.: 610%.

(E) An aqueous dispersion obtained by emulsion-polymerizing a composition consisting of 60% by weight of hexadecyl acrylate, 20% by weight of 2-ethylhexyl acrylate, 15% by weight of methyl acrylate and 5% by weight of hydroxyethyl acrylate. Static glass transition temperature: +4° C.

#### (4) An intermediate coating paint

(A) Amilac N-2 Sealer (an intermediate coating paint of amino polyester resin type manufactured by KANSAI PAINT CO., LTD.), pencil hardness at 20° C.: H

#### (5) Top coating paints

(A) Amilac White (a top coating color paint of amino alkyd resin type manufactured by KANSAI PAINT CO., LTD., a white paint for one coating and one baking) Pencil hardness at 20° C.: H

(B) Magicron Silver (a top coating metallic paint of amino acryl resin type manufactured by KANSAI PAINT CO., LTD., a silver metallic paint for two coatings and one baking) Pencil hardness at 20° C.: H

(C) Magicron Clear (a top coating clear paint of amino acryl resin type manufactured by KANSAI PAINT CO., LTD., a clear paint for two coatings and one baking) Pencil hardness at 20° C.: H

### II Examples and Comparative Examples

Using the above samples, there were conducted applications to metallic substrates, of cation type electrocoating paints, barrier coats, intermediate coating paints and top coating paints according to procedures shown in Table 1.

In Table 1, the conditions of cation electrodeposition were as follows: Solid content in bath: 20% by weight, bath temperature: 28° C., pH: 6.5, load voltage: about 250 V, electrification: about 180 sec. After electrocoating, water washing was conducted and then baking was conducted at 170° C. for 30 min. All film thicknesses are thicknesses after curing.

The barrier coats were applied using an air spray machine. All film thickness were 6 to 10  $\mu$  after drying at flat portions. Baking conditions 140° C., 30min.

The intermediate coating paints and the top coating paints were spray-coated using an electrostatic coating equipment. Baking conditions 140° C., 30min. Film thickness 20 $\mu$ .

In the top coating, "1C1B" refers to a coating system wherein a color paint is applied and then baked at 160° C. for 30 min. "2C1B" refers to a coating system wherein a metallic paint and a clear paint are applied in this order or a wet-on-wet basis and then the resulting two films are simultaneously baked at 160° C. for 30 min. All film thicknesses are for flat portions.

### III Results of Performance Tests

The coated panels obtained in the above Examples and Comparative Examples were used as test panels and subjected to performance tests. The results are shown in Table 2 which appears later.



TABLE 1-continued

|                          | Metallic substrate | Example |     |     | Comparative Example |     |     |      |     |     |
|--------------------------|--------------------|---------|-----|-----|---------------------|-----|-----|------|-----|-----|
|                          |                    | 17      | 18  | 19  | 1                   | 2   | 3   | 4    | 5   | 6   |
| Electro-coating          | Paint              | (A)     | (B) | (C) | (A)                 | (B) | (C) | (A)  | (B) | (C) |
| Film thickness ( $\mu$ ) |                    |         |     |     |                     |     |     |      |     |     |
| Flat portion             | 20                 | 20      |     |     |                     |     |     | 20   |     |     |
| Acute-angled portion     | —                  | 4       | 7   | —   | 4                   | 7   | —   | 4    | 7   |     |
| Barrier coating          | Paint              | (A)     | (B) | (C) |                     |     |     | —    |     | (E) |
| Intermediate coating     | Paint              |         | —   |     | (A)                 |     |     | —    |     | (A) |
| Top coating              | coating system     |         |     |     |                     |     |     | 2C1B |     |     |
| Paint name               |                    |         |     |     |                     |     |     | (B)  |     |     |
| Film thickness ( $\mu$ ) |                    |         |     |     |                     |     |     | 15   |     |     |
| Paint name               |                    |         |     |     |                     |     |     | (C)  |     |     |
| Film thickness ( $\mu$ ) |                    |         |     |     |                     |     |     | 35   |     |     |

TABLE 2

|                                              | Film | Example |     |     |     |     |     |     |     |     |     |     | Comparative Example |     |     |     |     |     | 14  | 15  | 16  | 17  | 18  | 19  | 1   | 2   | 3   | 4 | 5 | 6 | 7 |
|----------------------------------------------|------|---------|-----|-----|-----|-----|-----|-----|-----|-----|-----|-----|---------------------|-----|-----|-----|-----|-----|-----|-----|-----|-----|-----|-----|-----|-----|-----|---|---|---|---|
|                                              |      | 1       | 2   | 3   | 4   | 5   | 6   | 7   | 8   | 9   | 10  | 11  | 12                  | 13  | 14  | 15  | 16  | 17  | 18  | 19  | 1   | 2   | 3   | 4   | 5   | 6   | 7   |   |   |   |   |
| Chipping resistance                          | ○    | ○       | ○   | ○   | ○   | ○   | ○   | ○   | ○   | ○   | ○   | ○   | ○                   | ○   | ○   | ○   | ○   | ○   | ○   | ○   | ○   | ○   | ○   | ○   | ○   | ○   | ○   |   |   |   |   |
| Film surface condition                       | ○    | ○       | ○   | ○   | ○   | ○   | ○   | ○   | ○   | ○   | ○   | ○   | ○                   | ○   | ○   | ○   | ○   | ○   | ○   | ○   | ○   | ○   | ○   | ○   | ○   | ○   | ○   |   |   |   |   |
| Salt water spray resistance                  | ○    | ○       | ○   | ○   | ○   | ○   | ○   | ○   | ○   | ○   | ○   | ○   | ○                   | ○   | ○   | ○   | ○   | ○   | ○   | ○   | ○   | ○   | ○   | ○   | ○   | ○   | ○   |   |   |   |   |
| Impact resistance                            | ○    | ○       | ○   | ○   | ○   | ○   | ○   | ○   | ○   | ○   | ○   | ○   | ○                   | ○   | ○   | ○   | ○   | ○   | ○   | ○   | ○   | ○   | ○   | ○   | ○   | ○   | ○   |   |   |   |   |
| Adhesion                                     | 100  | 100     | 100 | 100 | 100 | 100 | 100 | 100 | 100 | 100 | 100 | 100 | 100                 | 100 | 100 | 100 | 100 | 100 | 100 | 100 | 100 | 100 | 100 | 100 | 100 | 100 | 100 |   |   |   |   |
| Water resistance                             | ○    | ○       | ○   | ○   | ○   | ○   | ○   | ○   | ○   | ○   | ○   | ○   | ○                   | ○   | ○   | ○   | ○   | ○   | ○   | ○   | ○   | ○   | ○   | ○   | ○   | ○   | ○   |   |   |   |   |
| Corrosion resistance at acute-angled portion | —    | —       | —   | —   | —   | —   | —   | —   | —   | —   | —   | —   | —                   | —   | —   | —   | —   | —   | —   | —   | —   | —   | —   | —   | —   | —   | —   |   |   |   |   |
| Salt water spray resistance                  | ○    | ○       | ○   | ○   | ○   | ○   | ○   | ○   | ○   | ○   | ○   | ○   | ○                   | ○   | ○   | ○   | ○   | ○   | ○   | ○   | ○   | ○   | ○   | ○   | ○   | ○   | ○   |   |   |   |   |
|                                              | Film | Example |     |     |     |     |     |     |     |     |     |     | Comparative Example |     |     |     |     |     |     |     |     |     |     |     |     |     |     |   |   |   |   |
|                                              |      | 14      | 15  | 16  | 17  | 18  | 19  | 1   | 2   | 3   | 4   | 5   | 6                   | 7   | 14  | 15  | 16  | 17  | 18  | 19  | 1   | 2   | 3   | 4   | 5   | 6   | 7   |   |   |   |   |
| Chipping resistance                          | ○    | ○       | ○   | ○   | ○   | ○   | X   | X   | X   | X   | X   | X   | Δ                   | Δ   | Δ   | Δ   | Δ   | Δ   | X   | X   | X   | X   | X   | X   | X   | X   | X   |   |   |   |   |
| Film surface condition                       | ○    | ○       | ○   | ○   | ○   | ○   | X   | X   | X   | X   | X   | X   | Δ                   | Δ   | Δ   | Δ   | Δ   | Δ   | X   | X   | X   | X   | X   | X   | X   | X   | X   |   |   |   |   |
| Salt water spray resistance                  | ○    | ○       | ○   | ○   | ○   | ○   | ○   | ○   | ○   | ○   | ○   | ○   | ○                   | ○   | ○   | ○   | ○   | ○   | ○   | ○   | ○   | ○   | ○   | ○   | ○   | ○   | ○   |   |   |   |   |
| Impact resistance                            | ○    | ○       | ○   | ○   | ○   | ○   | ○   | ○   | ○   | ○   | ○   | ○   | X                   | X   | X   | X   | X   | X   | ○   | ○   | ○   | ○   | ○   | ○   | ○   | ○   | ○   |   |   |   |   |
| Adhesion                                     | 100  | 100     | 100 | 100 | 100 | 100 | 100 | 100 | 100 | 100 | 100 | 100 | 100                 | 100 | 100 | 100 | 100 | 100 | 100 | 100 | 100 | 100 | 100 | 100 | 100 | 100 | 100 |   |   |   |   |
| Water resistance                             | ○    | ○       | ○   | ○   | ○   | ○   | ○   | ○   | ○   | ○   | ○   | ○   | ○                   | ○   | ○   | ○   | ○   | ○   | ○   | ○   | ○   | ○   | ○   | ○   | ○   | ○   | ○   |   |   |   |   |
| Corrosion resistance at acute-angled portion | ○    | ○       | ○   | —   | ○   | ○   | —   | —   | —   | —   | —   | —   | X                   | X   | X   | X   | X   | X   | —   | —   | —   | —   | —   | —   | —   | —   | —   |   |   |   |   |
| Salt water spray resistance                  | ○    | ○       | ○   | Δ   | ○   | Δ   | X   | X   | X   | X   | X   | X   | X                   | X   | X   | X   | X   | X   | X   | X   | X   | X   | X   | X   | X   | X   | X   |   |   |   |   |

## What we claim:

1. A process for coating a metallic substrate, which comprises applying on a metallic substrate an electro-coating paint, applying thereon a barrier coat comprising a film-forming thermoplastic resin other than a modified polyolefin resin and capable of forming a barrier coat film having a static glass transition temperature of  $-30^{\circ}$  to  $-60^{\circ}$  C. and an elongation at break of 300 to 800% in an atmosphere of  $-20^{\circ}$  C., said thermoplastic resin being at least one film-forming thermoplastic resin selected from the group consisting of styrene-butadiene copolymers, polybutadienes, acrylonitrile-butadiene copolymers, polybutenes, acrylic resins, natural rubber, polychloroprenes, methyl methacrylate-butadiene copolymers and polyvinylidene chlorides and then applying thereon a top coating paint, the film thickness of

the barrier coat being 1 to  $20\ \mu$  in terms of the thickness of the dried film, and the acrylic resins being copolymers of at least one monomer selected from the group consisting of acrylic esters and methacrylic esters, each of homopolymers of the acrylic esters and the methacrylic esters having a static glass transition temperature of  $0^{\circ}$  C. or lower, and the amount of these esters whose homopolymers have a static glass transition temperature of  $-40^{\circ}$  C. or lower constituting 60% by weight or more of the total monomer mixture.

2. The process according to claim 1, wherein the electrocoating paint is a thermosetting electrocoating paint of cathodic deposition type obtained by neutralizing a base resin having basic amino groups with an acid and dissolving or dispersing the resulting resin in water.

3. The process according to claim 1, wherein the electrocoating paint contains 35 parts by weight or less of pigments based on 100 parts by weight of resin solids.

4. The process according to claim 1, wherein the electrocoating paint contains 40 to 150 parts by weight, of pigments based on 100 parts by weight of resin solids.

5. The process according to claim 1, wherein the film-forming thermoplastic resin is at least one resin selected from the group consisting of styrene-butadiene copolymers and acrylic resins.

6. The process according to claim 1, wherein the film-forming thermoplastic resin is a styrene-butadiene copolymer having a styrene content of 1 to 80% by weight and a number-average molecular weight of 10,000 to 1,000,000 or an acrylic resin having a number-average molecular weight of 50,000 to 300,000 and comprising 30% by weight or more of an alkyl ester of acrylic acid or methacrylic acid whose homopolymer has a static glass transition temperature of -40° C. or less.

7. The process according to claim 1, wherein the barrier coat is an organic solvent or aqueous type paint.

8. The process according to claim 1, wherein the top coating paint is a top coating paint of amino acryl resin type or amino alkyd resin type.

9. The process according to claim 1, wherein the top coating paint is a paint capable of forming an ultra-hard coating film.

10. The process according to claim 9, wherein the ultra-hard coating film has a pencil hardness of 4H to 9H at 20° C. in terms of hardness of the cured film.

11. The process according to claim 1, wherein the top coating paint is directly applied on the barrier coat film.

12. The process according to claim 11, wherein the top coating paint has a powder form.

13. The process according to claim 12, wherein the barrier coat contains a compatible solvent.

14. The process according to claim 11, wherein the barrier coat contains at least one deterioration inhibitor for resins, selected from ultraviolet absorbers, photosensitizers and anti-oxidants.

15. The process according to claim 1, wherein the barrier coat further comprises a corrosion-preventive pigment.

16. The process according to claim 15, wherein an aqueous extract of the corrosion-preventive pigment contained in the barrier coat, has an electroconductivity of at least 100  $\mu$ /cm.

17. The process according to claim 15, wherein the barrier coat contains, per 100 parts by weight of the vehicle resin, 1-150 parts by weight of the corrosion-preventive pigment.

18. The process according to claim 15, wherein the corrosion-preventive pigment is selected from the group consisting of zinc chromate, strontium chromate, barium chromate and calcium chromate.

19. The process according to claim 1 wherein the static glass transition temperature is -40° to -55° C.

20. The metallic substrate coated according to a process of claim 1.

\* \* \* \* \*